

## UNITED STATES PATENT OFFICE

2,336,846

## ETCHING OF CAPACITOR ARMATURES

Frank M. Clark, Pittsfield, Mass., assignor to General Electric Company, a corporation of New York

No Drawing. Application January 3, 1938,  
Serial No. 183,131

6 Claims. (Cl. 204—141)

The present invention relates to the preparation of armatures for electric capacitors.

It is known that an improvement may be effected in electrolytic capacitors by etching the surface of their armatures. Etching materially increases the effective area of the exposed surface of the armatures and thereby correspondingly increases the capacity value for a given armature size.

Heretofore, it has been the practice to chemically etch the surface of capacitor metal by means of exposure to a solution of acid. When aluminum is subjected to such chemical etching, careful control is required of the various etching conditions, such for example, as acid concentration, temperature of reaction, and accumulation of by-products. When the material etched by such chemical process consists of aluminum foil, it is found that foil obtained from different sources reacts differently with a given acid etching bath. It is difficult to exercise this required close control in ordinary factory production. Even when the etching process is carried out under the supervision of highly skilled attendants, the tests and inspection which are required slows up the rate of production.

When it is attempted to replace the purely chemical etching procedure by electrolytic etching, the temperature, acidity and other conditions being so chosen that the removal of metal by ordinary chemical solution is substantially prevented, then deep cuts or scoring are produced in the surface of the metal being etched. As the metal armature stock commonly consists of thin foil, such cutting effect spoils or destroys the foil. Furthermore, it is difficult to completely remove the etching electrolyte from the deep cuts in the metal.

I have discovered that unexpectedly advantageous results are produced by etching armature metal by a combination of chemical and electrolytic action, the metal foil, or other armature material functioning as anode in an electrolytic bath which is capable also of producing ordinary chemical etching of metal at a slow rate. This combination effect produces an easily controlled shallow etching and not a deep scoring of the metal. When specifying aluminum chloride as an accelerator of acid activity in a claim for this invention I wish also to cover equivalent chlorides such as the chlorides of sodium and copper.

While the composition of the electrolytic bath and the conditions of electrolysis may be varied and should be governed by the character of the metal to be etched and other conditions, the fol-

lowing illustrative examples will illustrate my invention.

The etching electrolyte may consist of an aqueous solution of hydrochloric acid, an acid concentration well suited for etching purposes being about five per cent. Other electrolytic agents may be used as, for example, ammonium hydroxide, hydrofluoric acid, boric acid, sulphuric acid or acetic acid. However, hydrochloric acid is preferred. The metal to be etched, for example, aluminum foil, is caused to function as anode in such bath, the cathode conveniently consisting of carbon or other suitable inert conductive material. A bath temperature of 50 to 75° C. is suitable. A direct current having a density of about one-quarter ampere per square inch of active foil area and a voltage of about 4 to 6 volts may be impressed between the foil anode and the cathode in the electrolyte. Foil to be etched may be passed through the bath at such rate that a given area functions as anode in the electrolytic bath for two or three minutes.

When hydrochloric acid solution is used as the etching electrolyte, its activity is increased by the presence of about two to twelve per cent of metallic chlorides as, for example, sodium chloride, aluminum chloride and copper chloride. The content of aluminum chloride preferably should be maintained as low as about 6 per cent. When other acids are used for the etching electrolyte corresponding metallic salts preferably are present in about the same concentration.

After the etching step has been completed the etched metal is washed and oxidized in the usual way to produce a current-blocking oxide film, for example, by electrolysis in a solution of borax and boric acid as described in U. S. Patent No. 2,022,500 of Clark and Koenig, the etched foil functioning as anode.

If the etched and washed metal is to be stored before oxidation for any appreciable length of time, it preferably should be given immediately a low voltage anodic treatment to produce a light oxide film in order to prevent uncontrolled atmospheric oxidation which results in erratic capacity and power factor characteristic when the etched and oxidized armatures eventually are fabricated into capacitor units.

As a result of this conjoint electrolytic and non-electrolytic etching the rate of production of etched foil is materially increased, the consumption of acid per unit weight of metal acted upon is decreased and the uniformity of capacitors made from such etched armature foil is improved. In addition to such improvements the capacitors

made from such anodically etched foil possess a more stable capacity during periods of non-use, or as commonly stated during the "shelf life" period. The non-uniformities formerly noted in capacitors containing chemically etched armature foil obtained from different sources largely are eliminated.

What I claim as new and desire to secure by Letters Patent of the United States is:

1. The method of treating aluminum capacitor foil preparatory to producing a current-blocking film thereon which consists in immersing said foil in an aqueous reagent containing about 5 per cent hydrochloric acid and about 2 to 12 per cent of aluminum chloride, maintaining said reagent at a temperature of about 50 to 75° C., conducting between said foil functioning as anode and a cooperating cathode of carbon a direct current at a potential of about 4 to 6 volts and a density of about one-quarter ampere per square inch of active electrode surface, thereby causing etching by a combined chemical and electrolytic action, continuing said etching until the capacity value of the etched surface is effectively increased, and thereupon freeing said foil from said reagent.

2. The method of treating aluminum foil preparatory to producing a current-blocking film thereon for use in electrolytic capacitors which consists in introducing said foil into an electrolytic bath comprising an aqueous solution containing about 5 per cent of hydrochloric acid which is capable of producing chemical etching at a slow rate and approximately two to twelve per cent of aluminum chloride, impressing between said foil functioning as anode in said reagent and a cooperating cathode a direct current having at the active anode surface a density of about one-fourth ampere per square inch to increase the rate of etching, continuing such treatment for about two or three minutes for a given area to produce shallow etching without deep scoring of the etched metal surface and thereupon freeing said sheet from said reagent.

3. The method of treating aluminum foil preparatory to the formation of a current blocking film thereon which consists in introducing said foil into an aqueous reagent containing approximately 5 per cent hydrochloric acid, maintaining in said reagent approximately 2 to 12 per cent of an accelerator chosen from the group consisting of the chlorides of sodium, aluminum and copper, subjecting said foil to the anodic etching effect of an electric current between said foil and a cooperating electrode in said reagent thereby supplementing the chemical etching of said reagent,

continuing said treatment for a length of time sufficient to cause the resulting etching of said foil to increase the effective capacity value of the etched surface and thereupon freeing said foil from said reagent.

4. The method of treating aluminum foil preparatory to the formation of a current blocking film thereon which consists in introducing said foil into an etching electrolyte consisting essentially of an aqueous solution of hydrochloric acid of about 5 per cent concentration and about 6 per cent of aluminum chloride, subjecting said foil to the anodic etching effect of an electric current between said foil and a cooperating electrode in said electrolyte thereby supplementing the chemical etching effect of said electrolyte, continuing said treatment for a length of time sufficient to cause the resulting etching of said foil to increase the effective capacity value of the etched surface and thereupon freeing said foil from said electrolyte.

5. The method of treating aluminum foil preparatory to the formation of a current blocking film thereon which consists in introducing said foil into an etching electrolyte consisting essentially of an aqueous solution of hydrochloric acid of about 5 per cent concentration and about 2 to 6 per cent aluminum chloride, subjecting said foil to the anodic etching effect of an electric current between said foil and a cooperating electrode in said electrolyte thereby supplementing the chemical etching effect of said electrolyte, continuing said treatment for a length of time sufficient to cause the resulting etching of said foil to increase the effective capacity value of the etched surface and thereupon freeing said foil from said electrolyte.

6. The method of treating aluminum foil preparatory to the formation of a current blocking film thereon which consists in introducing said foil into an etching electrolyte consisting essentially of an aqueous solution of hydrochloric acid of about 5 per cent concentration and about 2 to 12 per cent of aluminum chloride, subjecting said foil to the anodic etching effect of an electric current between said foil and a cooperating electrode in said electrolyte thereby supplementing the chemical etching effect of said electrolyte, continuing said treatment for a length of time sufficient to cause the resulting etching of said foil to increase the effective capacity value of the etched surface and thereupon freeing said foil from said electrolyte.